

## UNITED STATES PATENT OFFICE

2,137,283

## COPPER ALLOYS

Franz R. Hensel and Earl I. Larsen, Indianapolis,  
Ind., assignors to P. R. Mallory & Co., Inc.,  
Indianapolis, Ind., a corporation of Delaware

No Drawing. Application August 12, 1938,  
Serial No. 224,499

1 Claim. (Cl. 75—159)

This invention relates to copper alloys. This case is a continuation in part of our co-pending application S. N. 164,032, filed September 15, 1937.

5 An object of the invention is to improve the physical, chemical and electrical characteristics of such alloys.

Other objects of the invention will be apparent from the following description, taken in connection with the appended claim.

The present invention comprises a combination of elements, methods of manufacture, and the product thereof, brought out and exemplified in the disclosure hereinafter set forth, the scope of 15 the invention being indicated in the appended claim.

While a preferred embodiment of the invention is described herein, it is contemplated that considerable variation may be made in the method 20 of procedure and the combination of elements, without departing from the spirit of the invention.

The present invention relates to the improvement of alloys of copper and zirconium. According to the present invention the improved 25 alloys are made of the following elements in substantially the following proportions:

|                                                                        | Per cent  |
|------------------------------------------------------------------------|-----------|
| 30 Metal selected from the group consisting of iron, cobalt and nickel | 0.1 to 30 |
| Zirconium                                                              | 0.05 to 5 |
| Beryllium                                                              | 0.05 to 3 |
| Copper                                                                 | balance   |

35 Where high electrical conductivities are desired, it is preferred to keep the proportion of iron group metal within an upper limit of 5%.

The alloys of the present invention may also contain small proportions, or even up to several 40 percent, of zinc, tin, calcium, lithium, magnesium, phosphorus and silver.

The beryllium combines with the iron group metal or metals to form the beryllide thereof and thereby imparts age-hardening characteristics to 45 the alloy.

The addition of zirconium in this type of alloy not only imparts additional age-hardening characteristics, but also produces a material of 50 corrosion resistance, high strength at elevated temperatures and superior fatigue and impact properties.

The alloys can be made according to standard alloying methods. A preferred method for introducing the zirconium is to prepare a hardener alloy 55 containing a high percentage of zirconium

and then introduce a predetermined amount of this alloy into a copper melt, containing the other ingredients in the desired proportions.

After the alloy has been prepared according to such methods, the material may be heat treated by first quenching the alloy in the form of a billet or sand casting, or any other form, from above 700° C. and subsequently aging at a temperature below 700° C. In certain cases, we have found it also advisable to use one heat 10 treatment only, namely, the low temperature treatment, and eliminate the quenching treatment.

If the materials are processed by rolling, extruding, drawing, forging or any other fabricating methods, we have found it desirable in many cases to quench the materials from the intermediate anneals, cold working same and applying an aging treatment afterwards. This cold working before aging hastens considerably the precipitation of the dispersed phase. In addition, a certain amount of cold work may be applied after aging in order to improve the surface finish of the wrought material.

An example of an alloy produced according to 25 the present invention is:

|           | Per cent |
|-----------|----------|
| Zirconium | 0.67     |
| Cobalt    | 2.04     |
| Silicon   | 0.63     |
| Copper    | balance  |

After quenching this alloy from 950° C. and aging at 450° C., a Rockwell B hardness of 105 was obtained, with an excess of 45% electrical conductivity. Cold working before or after aging had little effect on the hardness.

The addition of zirconium has further beneficial effects, in so far as it raises the annealing temperature, and at the same time provides a 40 very fine grain structure, which is highly desirable if the material is to be worked into sheets, strips, or tubing.

The composition which has exceptional merits for condenser tubing is as follows:

|           | Per cent  |
|-----------|-----------|
| Nickel    | 15 to 30  |
| Zirconium | 0.05 to 5 |
| Beryllium | 0.05 to 3 |
| Copper    | balance   |

While the present invention as to its objects and advantages has been described herein as carried out, in specific embodiments, it is not desired to be limited thereby, but it is intended to 55

cover the invention broadly within the appended claim.

What is claimed is:

5 A heat-treated alloy composed of 0.05 to 5% zirconium, 0.1 to 30% of a metal or a combination of metals selected from the group consisting of iron, cobalt and nickel, 0.05 to 3% beryl-

lium, and the balance substantially all copper, characterized by high hardness and further characterized by the fact that its hardness is not permanently adversely affected by temperatures in the order of 450° C.

FRANZ R. HENSEL.  
EARL I. LARSEN.